

## 1

3,429,673

## CORROSION INHIBITING ADDITIVE COMPOSITIONS FOR FUEL OILS

Günter Reese, Dusseldorf, and Günter Felletschin, Metzkausen über Mettmann, Germany, assignors to Henkel & Cie, G.m.b.H., Dusseldorf-Holthausen, Germany, a corporation of Germany  
 No Drawing. Filed Mar. 14, 1967, Ser. No. 622,922  
 Claims priority, application Germany, Apr. 5, 1966,  
 H 59,019

U.S. CL. 44—66  
 Int. CL. C10I 1/22, 1/18

11 Claims

## ABSTRACT OF THE DISCLOSURE

This invention relates to a corrosion inhibitor composition for fuel oils consisting of a mixture of:

(A) salts of aliphatic carboxylic acids having from 6 to 12 carbon atoms, with alkylamines substituted with hydroxyl groups; and  
 (B) salts of aliphatic carboxylic acids having from 4 to 12 carbon atoms, with alkylamines having from 4 to 16 carbon atoms, with the proviso that the total number of carbon atoms in said salt is more than 10;  
 said salts being present in said mixture in a ratio of 1:9 to 9:1 parts by weight. The invention also relates to fuel oils containing from 50 to 1000 parts per million of the aforesaid corrosion inhibitor composition.

## The prior art

The inner walls of the metal containers for the fuel oil supply are, as is well known, exposed to intense corrosion attacks. Primarily, these attacks are caused by water which enters the tank together with the fuel oil or possibly absorbed by the air which is drawn into the tank as the fuel oil is used. In any event this water tends to collect as a coherent layer on the bottom of the supply tank and as condensed moisture on the walls of this tank above the fuel oil level. Due to the fact that the oxygen present in this water is replenished continuously from the fuel oil during corrosion, this corrosion is advanced to a still greater degree. A further intensification of these corrosion attacks is caused by salts dissolved in the water, primarily chlorides, which get into the fuel oils in transportation and pass to the aqueous phase. The presence of salt-containing ground waters is even more dangerous, as they do not allow the presently known corrosion inhibiting agents, possibly present in the fuel oil, to take effect. Therefore, for some time, most types of fuel oils have been admixed with additives which are supposed to reduce the corrosive attacks.

As corrosion inhibitors organic nitrogen compounds, such as amines, have already been suggested, in particular long chain amines as well as alkanolamines, amides and their salts, also fatty acids or their salts. To some extent, these products guarantee good protection as long as the corrosion relates merely to an attack by condensation moisture or to corrosion due to salt-free ground water. To combat the attacks by salt-containing, in particular, chloride-containing solutions, the previously known fuel oil additives offer a sufficient protection only when disproportionately higher, frequently no longer economical, concentrations are employed.

## Objects of the invention

The object of the invention is to discover corrosion preventatives, in particular, corrosion inhibiting additives for fuel oils which guarantee, even in the presence of salt-containing, especially chloride-containing water, an espe-

## 2

cially pronounced protection already with the use of small amounts of the additives.

Another object of the invention is the obtention of a corrosion inhibitor composition for fuel oils consisting of a mixture of:

(A) salts of aliphatic carboxylic acids having from 6 to 12 carbon atoms, with alkylamines substituted with hydroxyl groups; and  
 (B) salts of aliphatic carboxylic acids having from 4 to 12 carbon atoms, with alkylamines having from 4 to 16 carbon atoms, with the proviso that the total number of carbon atoms in said salt is more than 10;

said salts being present in said mixture in a ratio of 1:9 to 9:1 parts by weight.

A further object of the invention is the obtention of a corrosion preventative fuel oil containing from 50 to 1000 parts per million of the aforesaid corrosion inhibitor composition.

These and other objects of the invention will become more apparent as the description thereof proceeds.

## Description of the invention

The invention accomplishes these objectives in that as corrosion preventatives, in particular corrosion inhibiting additives for fuel oils, such products are utilized which contain mixtures of:

(A) salts of aliphatic carboxylic acids having from 6 to 12 carbon atoms, with alkylamines substituted by hydroxyl groups; and  
 (B) salts of aliphatic carboxylic acids having from 4 to 12 carbon atoms, with alkylamines having from 4 to 16 carbon atoms, with the proviso that the total number of carbon atoms in said salt is more than 10;

said salts being present in said mixture in a ratio of 1 to 9 to 9 to 1.

In the case wherein salt A, carboxylic acids with 8 to 10 carbon atoms were used for the salt formation, a distinct improvement could be noted as compared with the shorter or longer chain acids. The use of carboxylic acids having from 6 to 10 carbon atoms as salt B can also be observed as an improvement compared with the shorter or longer chain acids. Among the amine components of the salt B, those having from 4 to 12 carbon atoms have the most favorable effect on the corrosion-preventing behavior. A further influence of the effectiveness of the salt mixture is possible by varying the proportions of the salts A and B in the total mixture. Here it became evident that the best results are obtained when the ratio of salt A to salt B fluctuates within the limits of 3:7 to 7:3 parts by weight.

Particularly effective mixtures are obtained when all improving factors are considered simultaneously. These preferred corrosion inhibitor compositions for fuel oils consist of a mixture of:

(A) salts of aliphatic carboxylic acids having from 8 to 10 carbon atoms, with alkylamines substituted by hydroxyl groups; and  
 (B) salts of aliphatic carboxylic acids having from 6 to 10 carbon atoms with alkylamines having from 4 to 12 carbon atoms, with the proviso that the total number of the carbon atoms in said salts is more than 10;

said salts being present in said mixture in a ratio of 3:7 to 7:3 parts by weight.

Suitable as acid components of the salt A are aliphatic carboxylic acids of natural origin, such as caproic acid, enanthic acid, caprylic acid, pelargonic acid, capric acid, undecanoic acid, lauric acid, and undecylenoic acid, and also synthetic carboxylic acids, as obtained by the paraffin oxidation or by addition of carbon monoxide and water to olefins. Generally, the above acids are alkanoic

acids and alkenoic acids having 6 to 12 carbon atoms. The best effectiveness may be attributed to the salts of caprylic, pelargonic and capric acids, of which caprylic acid (n-octanoic acid) is most outstanding.

The alkylamine component substituted by hydroxyl groups of the salt A can consist of monoethanolamine, diethanolamine, triethanolamine, propanolamine, isopropanolamine, triisopropanolamine, ethyleneoxide addition products of amines or alkanolamines, as for example, butylamine+3 ethylene oxide units, n-hexylamine+6 ethylene oxide units, 2-ethyl-hexylamine+6 ethylene oxide units, octylamine+8 ethylene oxide units, dodecylamine+12 ethylene oxide units, triethanolamine+2 ethylene oxide units, triethanolamine+6 ethylene oxide units, etc. The preferred alkylamine components of salt A are alkylamines containing hydroxyl groups of the formula



wherein  $R_1$ ,  $R_2$  and  $R_3$  are members selected from the group consisting of (a) hydrogen, (b) alkyl having from 1 to 12 carbon atoms (c) hydroxylalkyl having from 2 to 6 carbon atoms, and (d)  $-(CH_2-CH_2-O)_nH$ , where  $n$  is an integer of from 2 to 20, with the proviso that at least one of  $R_1$ ,  $R_2$  and  $R_3$  is selected from members (c) and (d) above. Triethanolamine was found to be the most suitable component.

As acid components of the salt B, butyric acid, valeric acid as well as those acids already indicated as acid components of the salts A can be used, of which caproic acid, enanthic acid, caprylic acid, pelargonic acid and capric acid seem to be especially appropriate. Generally the above acids are alcanoic acids and alkenoic acids having 4 to 12 carbon atoms. The very best results are obtained with caprylic acid.

As alkylamine components of salt B, butylamine, hexylamine, octylamine, decylamine, dodecylamine, hexadecylamine as well as amine mixtures as obtained, for example, from acids of corresponding chain length as occurring in natural oils and fats can be used. Preferably, these are mono-alkylamines having from 4 to 16 carbon atoms. Of the amines mentioned, those with short or medium length chains, as for example, butylamine, hexylamine,

octylamine, decylamine, and dodecylamine proved of better suitability. The best results were obtained with dodecylamine.

A mixture of triethanolamine-caprylate and dodecylamine-caprylate has been found the most favorable combination of all of the possibilities, absolutely suitable and furnishing very satisfactory results. Furthermore, this combination is the most effective when the mixture components are used at a ratio of 1:1.

10 The concentrations for use of the corrosion inhibitor salt mixtures of the invention, required for a sufficient protection in fuel oil, lies between 50 and 1000 p.p.m., based on fuel oil. Preferably, amounts of 100 to 250 p.p.m., based on fuel oil, are used.

15 The tests and the test results presented in the following serve for better comprehension of the objects of the invention. It is to be understood, however, that these embodiments are not to be deemed limitative in any respect.

### Examples

For the investigation of the effectiveness of the corrosion preventative compositions, rust-free, polished and degreased steel plates of the quality ST 37-2 (DIN 17.100), 2 mm. thick, 20 mm. wide and 100 mm. long, were placed in a standing cylinder of about 25 mm. diameter and 240 mm. height. Then 30 ml. of a pure unmixed fuel oil, to which various corrosion inhibitor salt mixtures had been added, and 3 ml. of an aqueous 0.3% sodium chloride solution were added. The steel plates were submerged about 6 mm. in the aqueous solution and were covered with oil up to a height of 60 mm. In this way, the rust development could be observed on all three boundary phases: water-steel, oil-steel and air-steel. The cylinders were kept locked for 7 days in the dark. Thereafter, the corrosion was judged visually and indicated with the numbers 0 to 10. The individual values were assigned the following significance:

0=unchanged appearance

1-3=slight corrosion

4-6=pronounced corrosion

7-10=very distinct corrosion.

The following table indicates the type of individual additions, the amounts of these, as well as the evaluation.

TABLE I.—ADDITION  
[p.p.m. based on fuel oil]

| Example | p.p.m. | Salt A                                               | p.p.m. | Salt B                   | Amount of corrosion |
|---------|--------|------------------------------------------------------|--------|--------------------------|---------------------|
| 1       | 0      | No addition                                          | 0      | No addition              | 10                  |
| 2       | 250    | Triethanolamine-caproate                             | 0      | Dodecylamine-caprylate   | 6                   |
| 3       | 0      |                                                      | 250    | do                       | 2                   |
| 4       | 125    | Triethanolamine-caproate                             | 125    |                          | 1                   |
| 5       | 250    | Triethanolamine-caprylate                            | 0      |                          | 3                   |
| 6       | 125    | do                                                   | 125    | Dodecylamine-caprylate   | 0                   |
| 7       | 250    | Triethanolamine-caprate                              | 0      |                          | 4                   |
| 8       | 125    | do                                                   | 125    | Dodecylamine-caprylate   | 0                   |
| 9       | 250    | Triethanolamine-laurate                              | 0      |                          | 5                   |
| 10      | 125    | do                                                   | 125    | Dodecylamine-caprylate   | 1                   |
| 11      | 250    | Monoethanolamine-caprylate                           | 0      |                          | 8                   |
| 12      | 125    | do                                                   | 125    | Dodecylamine-caprylate   | 1                   |
| 13      | 250    | Trisopropanolamine-caprylate                         | 0      |                          | 6                   |
| 14      | 125    | do                                                   | 125    | Dodecylamine-caprylate   | 1                   |
| 15      | 250    | 2-ethyl-hexyl-amine+6 ethylene oxide units-caprylate | 0      |                          | 8                   |
| 16      | 125    | do                                                   | 125    | Dodecylamine-caprylate   | 1                   |
| 17      | 250    | Dodecylamine+12 ethylene oxide units-caprylate       | 0      |                          | 8                   |
| 18      | 125    | do                                                   | 125    | Dodecylamine-caprylate   | 1                   |
| 19      | 0      |                                                      | 250    | Butylamine-caprylate     | 4                   |
| 20      | 125    | Triethanolamine-caprylate                            | 125    | do                       | 1                   |
| 21      | 0      |                                                      | 250    | Octylamine-caprylate     | 3                   |
| 22      | 125    | Triethanolamine-caprylate                            | 125    | do                       | 0                   |
| 23      | 0      |                                                      | 250    | Decylamine-caprylate     | 2                   |
| 24      | 125    | Triethanolamine-caprylate                            | 125    | do                       | 0                   |
| 25      | 0      |                                                      | 250    | Cocoamine-caprylate      | 2                   |
| 26      | 125    | Triethanolamine-caprylate                            | 125    | do                       | 0                   |
| 27      | 0      |                                                      | 250    | Hexadecylamine-caprylate | 5                   |
| 28      | 125    | Triethanolamine-caprylate                            | 125    | do                       | 2                   |
| 29      | 0      |                                                      | 250    | Dodecylamine-butyrate    | 3                   |
| 30      | 125    | Triethanolamine-caprylate                            | 125    | do                       | 1                   |
| 31      | 0      |                                                      | 250    | Dodecylamine-caproate    | 2                   |
| 32      | 125    | Triethanolamine-caprylate                            | 125    | do                       | 0                   |
| 33      | 0      |                                                      | 250    | Decylamine-caprate       | 2                   |
| 34      | 125    | Triethanolamine-caprylate                            | 125    | do                       | 0                   |
| 35      | 0      |                                                      | 250    | Dodecylamine-caprate     | 3                   |

See footnotes at end of table.

TABLE I.—Continued  
[p.p.m. based on fuel oil]

| Example | p.p.m. | Salt A                    | p.p.m. | Salt B                 | Amount of corrosion |
|---------|--------|---------------------------|--------|------------------------|---------------------|
| 36      | 125    | Triethanolamine-caprylate | 125    | do                     | 0                   |
| 37      | 0      | do                        | 250    | Dodecylamine-laurate   | 4                   |
| 38      | 125    | Triethanolamine-caprylate | 125    | do                     | 1                   |
| 39      | 50     | do                        | 50     | Dodecylamine-caprylate | 1                   |
| 40      | 25     | do                        | 25     | do                     | 2                   |
| 41      | 25     | Triethanolamine caproate  | 225    | do                     | 2                   |
| 42      | 225    | do                        | 25     | do                     | 4                   |
| 43      | 150    | do                        | 100    | do                     | 2                   |
| 44      | 100    | do                        | 150    | do                     | 2                   |
| 45      | 50     | do                        | 450    | do                     | 1                   |

<sup>1</sup> Coccamine is the mixed amine derived from coconut oil fatty acids.

As it can be concluded from the preceding Table I, the individual salts already reduce the corrosive effect of the aqueous phase in the fuel oil to a certain degree when used by themselves. (See Examples 2, 3, 5, 7, 9, 11, 13, 15, 17, 19, 21, 23, 25, 27, 29, 31, 33, 35 and 37.) However, if the corrosion inhibitor mixtures of the invention are used, a substantially greater protection is obtained than that which was to be expected from the total of the individual effects of the two components of the mixture. This synergistic effect makes it possible to obtain a fully satisfactory corrosion protective effect against aqueous, chloride-containing solutions with low concentrations of use of the corrosion inhibitor compositions of the invention.

To gain further information concerning the effectiveness of the fuel oil additives of the invention, a quantitative test was conducted according to the specifications given by the Eidgenössischen Metallprüfungs und Versuchsanstalt (Federal Metal Testing and Research Institute) (EMPA-Publications 2/1964).

A square, rust-free, polished, degreased steel plate (ST 35 37-2, DIN 17,100) of known weight and 2 mm. thickness with a length of 20 mm., was placed in a 50 ml. beaker. 45 ml. of fuel oil was poured over the steel plate, and while vigorously stirring, 0.23 ml. of water or 0.23 ml. of sodium chloride solutions having a concentration 40 varying from 0.3% to 3% were added. The aqueous phase settled gradually in drops on the steel plate and produced a corresponding corrosion. The beakers, covered with a watch glass, were allowed to stand in the dark for 28 days. Thereafter, the rust formed was carefully scraped off with cellulose and the steel plate was again weighed after having been dried. The loss of iron was ascertained from the difference and converted into gram of loss of iron/m.<sup>2</sup> of surface. The values thus obtained 45 are reported in the following table.

15 nique. Moreover, with the use of the corrosion preventative compositions of the invention, no foreign substances which could have an unfavorable effect during the combustion of the fuel oil in the boiler are added to the fuel oil.

20 The preceding specific embodiments are illustrative of the invention. It is to be understood, however, that other expedients known to those skilled in the art can be employed without departing from the spirit of the invention or the scope of the appended claims.

25 We claim:

1. An aqueous sodium chloride corrosion inhibitor composition for fuel oils consisting of a mixture of  
(A) salts of aliphatic carboxylic acids containing from 8 to 10 carbon atoms selected from the group consisting of alcanoic acids and alkenoic acids, with alkylamines containing hydroxyl groups of the formula



30 wherein R<sub>1</sub>, R<sub>2</sub> and R<sub>3</sub> are members selected from the group consisting of (a) hydrogen, (b) alkyl having from 1 to 12 carbon atoms, (c) hydroxyalkyl having from 2 to 6 carbon atoms, and (d)



35 where n is an integer from 2 to 20, with the proviso that at least one of R<sub>1</sub>, R<sub>2</sub> and R<sub>3</sub> is selected from members (c) and (d) above; and

(B) salts of aliphatic carboxylic acids containing from 6 to 10 carbon atoms selected from the group consisting of alcanoic acids and alkenoic acids, with monoalkylamines having from 4 to 12 carbon atoms, with the proviso that the total number of carbon atoms in said salt is more than 10;

TABLE II

| Example | Triethanol-amine-caprylate (p.p.m. in the fuel oil) | Dodecyl-amine-caprylate (p.p.m. in the fuel oil) | G. of iron loss/m. <sup>2</sup> of surface |      |       |
|---------|-----------------------------------------------------|--------------------------------------------------|--------------------------------------------|------|-------|
|         |                                                     |                                                  | H <sub>2</sub> O                           | 0.3% | 1.0%  |
| 46      | 0                                                   | 0                                                | 35                                         | 63   | 97    |
| 47      | 125                                                 | 125                                              | 0                                          | 0    | 108   |
| 48      | 75                                                  | 75                                               | -----                                      | 0    | ----- |
| 49      | 25                                                  | 25                                               | -----                                      | 0    | ----- |

50 From the figures indicated in Table II, the outstanding corrosion inhibiting effect of the triethanolamine-caprylate/dodecylamine-caprylate mixtures can be seen even in the presence of greater sodium chloride concentrations which might be present in the ground water. These inhibiting effects occur even at extremely low concentrations of the corrosion inhibitor compositions of the invention in fuel oil.

The advantage obtainable according to the invention consists in that with even low concentrations of the indicated salt mixtures in fuel oil, a complete protection can be obtained for the storage tank against corrosion due to salt-containing water. Particularly, the salt-containing waters have until now caused the greatest difficulties with respect to the corrosion preventative tech-

65 to 7:3 parts by weight.

2. The aqueous sodium chloride corrosion inhibitor composition for fuel oils of claim 1, wherein the carboxylic acid component of the salt A is an alcanoic acid having 8 to 10 carbon atoms.

3. The aqueous sodium chloride corrosion inhibitor composition for fuel oils of claim 1, wherein the carboxylic acid component of the salt B is an alcanoic acid having 6 to 10 carbon atoms.

4. The aqueous sodium chloride corrosion inhibitor composition for fuel oils of claim 1 wherein the carboxylic acid component of salt A is caprylic acid.

5. The aqueous sodium chloride corrosion inhibitor composition for fuel oils of claim 1 wherein the alkyl-

amine containing hydroxyl group component of salt A is triethanolamine.

6. The aqueous sodium chloride corrosion inhibitor composition for fuel oils of claim 1 wherein the carboxylic acid component of salt B is caprylic acid.

7. The aqueous sodium chloride corrosion inhibitor composition for fuel oils of claim 1 wherein the mono-alkylamine component of salt B is dodecylamine.

8. The aqueous sodium chloride corrosion inhibitor composition for fuel oils of claim 1 wherein salt A is triethanolamine-caprylate, salt B is dodecylamine-caprylate and said salts A and B are present in a ratio of 1 to 1 parts by weight.

9. Fuel oil containing from 50 to 1000 parts per million, based on the fuel oil of the aqueous sodium chloride corrosion inhibitor composition for fuel oils of claim 1.

10. Fuel oil containing from 50 to 1000 parts per million, based on the fuel oil of the aqueous sodium chloride corrosion inhibitor composition for fuel oils of claim 8.

11. Fuel oil containing from 100 to 250 parts per

million, based on the fuel oil of the aqueous sodium chloride corrosion inhibitor composition for fuel oils of claim 1.

## References Cited

## UNITED STATES PATENTS

|           |         |               |         |    |
|-----------|---------|---------------|---------|----|
| 1,990,365 | 2/1935  | Beale         | 44-66   | XR |
| 2,382,818 | 8/1945  | Rhodes et al. | 252-392 | XR |
| 2,433,243 | 12/1947 | Smith et al.  | 44-66   |    |
| 2,587,546 | 2/1952  | Matuszak      | 252-392 | XR |
| 2,614,980 | 10/1952 | Lytle         | 252-392 | XR |
| 2,736,658 | 2/1956  | Pfohl et al.  | 44-66   | XR |
| 2,798,045 | 7/1957  | Buck et al.   | 44-71   | XR |
| 2,939,842 | 6/1960  | Thompson      | 44-71   | XR |

DANIEL E. WYMAN, Primary Examiner.

WILLIAM J. SHINE, Assistant Examiner.

U.S. CL. X.R.

44-71